

## UNITED STATES PATENT OFFICE

2,301,360

PURIFICATION OF HIGH SILICON IRON  
ALLOYSJoseph H. Brennan, Niagara Falls, N. Y., assignor  
to Electro Metallurgical Company, a corpora-  
tion of West VirginiaNo Drawing. Application August 3, 1940,  
Serial No. 351,125

3 Claims. (Cl. 75—53).

This invention relates to the purification of molten silicides and alloys containing a large proportion of silicon and refers more particularly to a process of removing calcium and aluminum from such molten silicides and alloys.

The raw materials used in the production of silicides and such alloys as ferrosilicon frequently contain alumina and lime as impurities, and when the usual manufacturing processes are pursued, using such materials, the silicides or alloys produced are contaminated with aluminum and calcium. There is a demand, notably in the production of electrical steel sheet, for silicides and high silicon alloys practically free from such contaminants, and to achieve the desired purity it has heretofore been necessary to use very pure grades of raw materials. These special raw materials are more expensive than the ordinary materials utilized, and there is a demand for a method utilizing cheaper grades of raw materials but at the same time producing silicides or high silicon alloys containing little or no aluminum or calcium. It is a principal object of this invention to provide such a method.

This object is achieved by the invention which comprises adding to a molten high silicon alloy or silicide produced in the usual way from the usual raw materials a quantity of a metal sulphide sufficient to remove aluminum and calcium. A preferred material for refining aluminum and calcium from high silicon alloys is iron pyrites. If iron is an objectionable impurity in the alloy or silicide being produced, nickel sulphide or cobalt sulphide or other appropriate sulphide may be employed. The sulphide may be added to the molten silicide or alloy either in the ladle or in an auxiliary refining furnace. In either event aluminum and calcium are removed in a fluid slag, probably as aluminum and calcium sulphides. Under properly controlled conditions, there is no substantial loss of silicon incurred in the treatment of the invention, and moreover, the sulphur content of the material treated is not increased to any important degree.

The amount of sulphide to be used in the method of the invention is dependent on the proportions of aluminum and calcium present in the material to be treated and on how much of the impurities is to be removed as well as on the conditions of operation. When iron pyrites is used, the quantity to be added may be based on the equations:



In the practice of the invention the sulphide treatment is preferably carried out in the ladle. Thus, a silicide or high silicon alloy is produced in the usual way, and a part of it may then be tapped into a ladle. The desired amount of sulphide is added to the material in the ladle, and the remainder of the silicide or alloy is then tapped rapidly to provide a stirring action. The molten material in the ladle is allowed to cool to proper pouring temperature. The sulphide treatment apparently raises the temperature of the material in the ladle and a longer time is necessary for cooling than is necessary when no sulphide addition is made, but this longer cooling period is advantageous because it insures completion of the refining action of the sulphide before pouring.

The following specific examples of the application of the method of the invention to the refining of ferrosilicon illustrate the principles and practice of the invention. It is to be understood, however, that the invention is not limited to the treatment of ferrosilicon but is equally applicable to the refining of other high silicon alloys or silicides.

Two hundred and fifty pounds of iron pyrites containing about 41% iron and 48% sulphur, the remainder principally silica, were added to the ladle during the tapping of about 7500 pounds 30 of ferrosilicon containing 47.16% silicon, 1.5% aluminum, 0.08% calcium, 0.003% sulphur, remainder principally iron. The molten ferrosilicon was tapped rapidly to give a good stirring action. The molten material in the ladle was 35 allowed to cool to a low pouring temperature and was then poured into chills. The ferrosilicon produced contained 47.23% silicon, 1.07% aluminum, 0.006% sulphur and nil calcium. Thus, the silicon to aluminum ratio was improved from 40 31.4 to 1 to 44.2 to 1, there was no loss of silicon, no appreciable increase in sulphur content, and the calcium was entirely eliminated.

In another test of the method of the invention 6500 pounds of a molten ferrosilicon containing 50.65% silicon, 1.45% aluminum, 0.26% calcium, 0.005% sulphur, the remainder principally iron, were tapped into a ladle. A portion of the molten ferrosilicon was then poured from this 45 ladle into a second ladle and 275 pounds of iron pyrites containing about 41% iron and 48% sulphur were rapidly added to the small portion of molten metal in the second ladle. The remaining ferrosilicon in the first ladle was then poured into the second ladle, the stream stirring the 50 material already in the second ladle. After all of

the ferrosilicon had been poured into the second ladle, the contents of the second ladle were repoured into the first ladle to obtain further stirring. The molten metal was then allowed to cool to pouring temperature and was then poured into chills. The product contained 49.84% silicon, 0.73% aluminum, 0.02% calcium and 0.003% sulphur. Thus, by the sulphide treatment the aluminum in the ferrosilicon was decreased from 1.45% to 0.73%, the calcium was decreased from 0.26% to 0.02%, there was no increase in sulphur content, and the silicon content was not substantially decreased.

In another test of the method of the invention 250 pounds of iron pyrites of the same lot used in the previous examples were added to a ladle containing 7000 pounds of a ferrosilicon containing 0.8% aluminum and 0.07% calcium. After the pyrites treatment the ferrosilicon produced contained 0.34% aluminum and 0.01% calcium. In still another test the aluminum content of 7000 pounds of ferrosilicon was reduced from 0.59% to 0.19% and the calcium content of 0.01% in the ferrosilicon was entirely eliminated by adding 500 pounds of iron pyrites to the ladle.

The treatment of the invention may be carried out in a furnace as well as in the ladle. In one test 300 pounds of ferrosilicon containing about 50% silicon were treated with 36 pounds of iron pyrites containing about 41% iron and 48% sulphur in an electric furnace. The aluminum content of the ferrosilicon was reduced from 0.39% to 0.19% and the calcium content was reduced from 0.06% to 0.04%.

It has been found that high silicon alloys or silicides which have been given the sulphide

treatment of the invention not only contain less aluminum and calcium than alloys or silicides which have not been given this treatment, but the material produced is exceptionally sound and dense and is considerably tougher than alloys or silicides which have not been given the treatment of the invention.

While specific examples have been given of the application of the invention to the production of ferrosilicon these examples merely illustrate the principles of the invention and the invention is not limited to such examples. For instance, it may be used to advantage in the treatment of nickel-silicon alloys, cobalt-silicon alloys, and other high silicon alloys or silicides.

I claim:

1. A process of purifying iron alloys containing a large proportion of silicon and only small proportions of the impurities aluminum and calcium which comprises subjecting a molten bath of such high silicon alloy to the action of a metallic sulphide.

2. A process of preparing ferrosilicon containing unobjectionable proportions of aluminum and calcium which comprises subjecting a molten ferrosilicon containing objectionable proportions of such elements to the action of iron sulphide.

3. A process of preparing a ferrosilicon containing unobjectionable proportions of aluminum and calcium as impurities which comprises forming a molten bath of a ferro-silicon containing objectionable proportions of such elements and adding to such bath a quantity of iron sulphide sufficient to remove at least a portion of the aluminum and calcium present in said ferrosilicon.

JOSEPH H. BRENNAN.